

## UNITED STATES PATENT OFFICE

1,959,399

## STEEL AND PROCESS OF MAKING SAME

John Thomas Whiteley, Dunellen, N. J., assignor  
to Isack W. Heyman and Sol L. Zavon, co-  
partners trading as Multi Steel Co., New York,  
N. Y.

No Drawing. Application February 25, 1932,  
Serial No. 595,220

19 Claims. (Cl. 75—1)

The present invention relates to steel and its manufacture and to the purification of iron.

For many years it has been the dream of steel makers to produce a commercially satisfactory steel without the aid of carbon or with only very small proportions of carbon. Carbon has the notable and valuable property of hardening iron but it also has a tendency to make it brittle and the desire of the steel maker is to produce a steel that is not only very hard but also one that has improved mechanical strength and toughness.

The present invention provides the solution to the problem hereinabove referred to.

The invention is in part based upon the discovery that a far reaching improvement occurs when certain agents apparently having a catalytic action are added to an iron melt containing zirconium and titanium. It is the combined use of zirconium and titanium, on the one hand and a suitable catalytic agent on the other hand that brings about the desired result. The theory that may explain the mechanism of the reaction is as follows:

Zirconium and titanium act as reducing agents i. e. deoxidizing agents on the oxide impurities in the iron. Their action is however, incomplete and sluggish. When a suitable catalyst is employed however, an extremely vigorous and complete purifying reaction sets in resulting in a substantially complete union of the oxygen impurities with the zirconium and titanium. This theory is substantiated by the fact that only enough zirconium and titanium e. g. from 0.2 to 0.5 per cent of each, is necessary, in conjunction with the catalyst, to effect the desired result. The theory that the zirconium and titanium, aided by the catalytic agent, exert a purifying action on the low carbon iron is further substantiated by a microscopical examination of the final product produced, as for example, according to Examples 1 or 2 below. The structure is found to be extremely close grained and homogeneous and free from inclusions and segregations.

But whatever the theory may be, the fact remains that the use of a trace of certain materials (which for want of a better name will be termed catalysts) causes some chemical reaction to occur between the zirconium and titanium and the iron melt and this reaction produces steel with a greatly improved hardness and toughness even though the carbon content is extremely low, for example, less than 0.5 per cent and even as low as 0.05 per cent.

The preferred catalyst is a bichromate e. g. sodium bichromate but other strong oxidizing agents may be used for example, potassium bichromate, potassium chlorate, sodium nitrate,

potassium permanganate, sodium perborate, etc. These examples will suffice to show that any powerful oxidizing agent may be used.

The present invention is not therefore a mere slight improvement in a crowded art, not a narrow portion of a broad field already staked out by prior inventors. So far as known, no one ever suggested or thought of the idea of using an oxidizing agent to effect deoxidation and yet that is just what the present invention apparently does. It may be and is believed that the trace of oxidizing agent added activates the zirconium and titanium to exert the full extent of their deoxidizing powers. Whatever the theory may be, it is a fact that the trace of oxidizing agent is the key that unlocks the power of the deoxidizing agent to confer on the iron melt the remarkable properties of toughness and hardness possessed by steel made according to the present invention.

If the theory herein advanced is the correct one, then the seemingly paradoxical fact exists that the addition of a strong oxidizing agent facilitate the removal or abstraction of oxygen from the melt. This can be explained chemically on the hypothesis that the oxygen impurities exist in the steel in the form of non-volatile metallic oxides which may be reduced by titanium and zirconium, i. e. the titanium and zirconium activated by the catalyst or strong oxidizing agent unite with the oxygen of the oxide impurities to form oxides of zirconium and titanium. The latter are volatile and pass off as smoke or vapor at the high temperature at which the reaction is carried out. But it is the trace of strong oxidizing agent e. g. sodium bichromate which initiates and maintains the reaction between the titanium and zirconium on the one hand and the oxide impurities on the other. The trace or small quantity of added oxidizing agent or catalyst acts on the titanium and zirconium and spurs them into a state of activity. Having once attained this activated condition, the zirconium and titanium then proceed to abstract oxygen from the oxide impurities. This theory of the mechanism of the reaction is substantiated by the observed fact that although zirconium and titanium are added to the melt, they do not appear in the final finished steel, (at least not in the proportions introduced) indicating that they are converted into a volatile compound or oxide which passes off as a vapor or smoke.

The invention will be illustrated by a typical example as follows.

Pig iron is refined, as by Bessemerizing, down to a carbon content of 0.20 to 0.50 per cent e. g.

0.30 per cent. It is then brought to a temperature of about 2800° F. and the following ingredients added in the proportion named.

*Example 1*

|            | Per cent     |
|------------|--------------|
| Molybdenum | 0.40 to 0.75 |
| Chromium   | 0.10 to 0.30 |
| Silicon    | 0.20 to 0.50 |
| Manganese  | 0.50 to 1.00 |

10 Zirconium (0.50%) and titanium (0.20%) are now incorporated and the melt is stirred to thoroughly mix and dissolve the added components.

15 A trace of sodium bichromate is now added and stirred in and immediately a vigorous reaction ensues, the temperature of the melt increases spontaneously and smoke is produced. Upon analyzing the resulting product, substantially no zirconium or titanium is found.

20 The molybdenum, silicon, manganese and chromium cooperate with the iron or low-carbon steel purified by the zirconium-titanium-oxidizing agent reaction to produce a steel having a remarkable combination of hardness and toughness; and to still further increase these properties especially in the direction of toughness, nickel and copper are added. The preferred proportion of nickel is 0.10 to 0.35 per cent and of copper 0.50 to 0.90 per cent. One of the especially desirable properties of a steel produced as described is that it requires no tempering to develop its toughness and hardness and it may be safely quenched in water or oil from about 1700° F. without a subsequent tempering. For example, an expensive die can be quenched without cracking and is then ready for use without tempering.

25 I have found that by employing tungsten and vanadium (and also preferably a trace of boron and cobalt) in addition to the elements already named in Example 1 above and otherwise proceeding generally as set forth therein, that the carbon content can be reduced below 0.30 per cent and in a typical case illustrating this phase of the invention I proceed as follows:

30 45 A charge of pig iron is purified, as for example by Bessemerizing, until the carbon content is very low, for example 0.10 per cent and to this is added at about 2800° F.;

*Example 2*

|              | Per cent     |
|--------------|--------------|
| Molybdenum   | 0.75 to 1.50 |
| Manganese    | 0.80 to 1.20 |
| Silicon      | 0.80 to 1.20 |
| Chromium     | 0.50 to 1.00 |
| 55 Tungsten  | 0.30 to 0.60 |
| Vanadium     | 0.10 to 0.20 |
| Cobalt       | a trace      |
| Boron        | a trace      |
| also         |              |
| 60 Zirconium | 0.20 to 0.50 |
| Titanium     | 0.20 to 0.50 |

65 When thorough distribution of these metals has occurred, a trace of a powerful oxidizing catalyst e. g., a bichromate of which sodium bichromate is a typical example, is added whereupon a vigorous reaction takes place. When this has subsided, the charge is poured off and allowed to cool in the form of ingots, etc.

70 75 According to this phase of the invention, the carbon may be eliminated entirely and in no case is it necessary to exceed approximately 0.20 per cent.

To further aid in developing toughness, I employ copper (0.30 to 7.00 per cent) and nickel

(0.50 to 1.00 per cent) in combination with the elements set forth in Example 2.

This application is a continuation in part of my copending applications Serial No. 334,856 filed January 24, 1929, and Serial No. 413,136 filed December 10, 1929.

80 85 The steel produced according to the present invention is further differentiated from other steels in that it consists mostly of iron the minimum proportion of which is of the order of 85 per cent. It does not contain the excessive quantities of expensive elements now commonly used in making alloy steels and the reason why I am enabled to attain a steel having the properties set forth is to be ascribed in my opinion to a peculiar crystalline structure created by the potent effects of the zirconium and titanium in conjunction with the catalytic agent. Therefore, the steel produced according to the present invention is economical to produce and in steel manufacture, economy is vital.

90 95 Certain very specific percentages of elements have been set forth but it is to be clearly understood that these are illustrative only and that the invention in its broader aspects is not limited by such specific proportions. Having set forth the principles of the invention and provided certain clear and concise examples of how it may be practised, those skilled in the art will be able to vary the proportions and make other changes 100 105 without going beyond the true scope of the invention which is intended to be defined by the appended claims.

What I claim is:

1. The method of treating iron which comprises melting it, adding zirconium and titanium and then initiating an exothermic reaction by adding a powerful oxidizing agent selected from the group consisting of sodium bichromate, potassium bichromate, potassium chlorate, sodium nitrate, potassium permanganate and sodium perborate.

110 115 2. The method of purifying iron which comprises melting it, incorporating zirconium and titanium and initiating a vigorous reaction between oxide impurities and said zirconium and titanium by adding a powerful oxidizing agent selected from the group consisting of sodium bichromate, potassium bichromate, potassium chlorate, sodium nitrate, potassium permanganate and sodium perborate.

120 125 3. The method of making steel which comprises heating it to a high temperature, incorporating therewith zirconium and titanium and also molybdenum, manganese, silicon and chromium, and adding a powerful oxidizing agent selected from the group consisting of sodium bichromate, potassium bichromate, potassium chlorate, sodium nitrate, potassium permanganate and sodium perborate which initiates a 130 135 vigorous reaction between the zirconium and titanium and oxide impurities.

140 145 4. The method of making steel which comprises heating to a high temperature a batch of iron having not more than 0.5 per cent carbon, incorporating therewith zirconium and titanium and also molybdenum, manganese, silicon and chromium and adding a powerful oxidizing agent selected from the group consisting of sodium bichromate, potassium bichromate, potassium chlorate, sodium nitrate, potassium permanganate and sodium perborate which initiates a 150 155 vigorous reaction between the zirconium and titanium and oxide impurities.

5. The method of making steel which com-

- prises heating to a high temperature a batch of iron having not more than 0.2 per cent carbon, incorporating therewith zirconium and titanium and also molybdenum, manganese, silicon, chromium, tungsten, vanadium, boron and cobalt, and adding a powerful oxidizing agent selected from the group consisting of sodium bichromate, potassium bichromate, potassium chlorate, sodium nitrate, potassium permanganate and sodium perborate which initiates a vigorous reaction between the zirconium and titanium and oxide impurities. 5
6. An alloy steel comprising molybdenum 0.40 per cent to 0.75 per cent, chromium 0.10 to 0.30 per cent, silicon 0.20 to 0.50 per cent, manganese 0.5 to 1.0 per cent and the balance substantially iron, said steel having been treated in the molten condition with zirconium, titanium and sodium bichromate. 10
7. An alloy steel having a lower carbon content of 0.2 to 0.5 per cent and the balance substantially iron, said steel having been treated in the molten condition with sodium bichromate, zirconium and titanium. 20
8. An alloy steel containing carbon 0.2 to 0.5 per cent, molybdenum 0.40 to 0.75 per cent, nickel 0.10 to 0.35 per cent, copper 0.50 to 0.90 per cent, chromium 0.10 to 0.30 per cent, manganese 0.50 to 1.00 per cent and the balance 25 substantially iron and deoxidized by zirconium, titanium and an oxidizing salt selected from the group consisting of sodium bichromate, potassium bichromate, potassium chlorate, sodium nitrate, potassium permanganate and sodium perborate. 30
9. An alloy steel containing carbon 0.20 to 0.50 per cent, molybdenum 0.40 to 0.75 per cent, nickel 0.10 to 0.35 per cent, silicon 0.20 to 0.50 per cent, copper 0.50 to 0.90 per cent, chromium 0.10 to 0.30 per cent, manganese 0.50 to 1.00 per cent and the balance 35 substantially iron and deoxidized by zirconium, titanium and sodium bichromate. 40
10. A deoxidized alloy steel containing 0.2 to 0.5 per cent carbon and the balance substantially iron deoxidized by reaction with zirconium 0.5 to 1.5 per cent, 0.1 to 0.3 per cent titanium and a chromate oxidizing salt. 45
11. The process of making a hardened and ductile steel comprising treating a quantity of iron with carbon in the proportion of from 0.2 to 0.5 per cent and adding to the melt zirconium, titanium and sodium bichromate at such intervals that they enter into a reaction with one another. 50
12. The process of making a hardened and ductile steel comprising treating a quantity of iron with carbon in the proportion of from 0.2 to 0.5 per cent and adding to the melt zirconium, titanium and a chromate oxidizing agent at such intervals that they enter into a reaction with one another. 60
13. The process of making steel which comprises treating a quantity of iron with carbon in the proportion of from 0.2 to 0.5 per cent, treating the melt with molybdenum, manganese, silicon and chromium and adding thereto zirconium, titanium and a bichromate at such intervals that they enter into a reaction with one another. 65
14. The process of making a hardened and ductile steel comprising treating a quantity of iron with carbon in the proportion of from 0.2 to 0.5 per cent, treating the melt with molybdenum, nickel, silicon, copper, chromium, manganese and adding thereto zirconium and titanium and a bichromate oxidizing agent at such intervals that they enter into a reaction with one another. 70
15. The process of making a hard tough steel containing carbon in an amount substantially between 0.2 and 0.5 per cent which comprises treating iron at a high temperature with substantially 0.2 to 0.5 per cent carbon, adding zirconium and titanium to deoxidize impurities of the iron and initiating a deoxidizing reaction between the said oxide impurities and the zirconium and titanium by incorporating a trace of a chromate oxidizing agent, whereby the steel is rendered homogeneous. 80
16. The method of treating iron having a carbon content not greater than 0.5 per cent which comprises melting it with copper 0.3 to 7.0 per cent, nickel 0.1 to 0.35 per cent, molybdenum 0.75 to 1.5 per cent, chromium 0.5 to 1.0 per cent, manganese 0.8 to 1.2 per cent, tungsten 0.3 to 0.6 per cent, cobalt a trace, boron a trace, adding zirconium and titanium to the melt and then initiating a combination of the oxide impurities with the zirconium and titanium by the addition of an oxidizing agent selected from the group consisting of sodium bichromate, potassium bichromate, potassium chlorate, sodium nitrate, potassium permanganate and sodium perborate. 85
17. The method of treating iron having a carbon content not greater than 0.5 per cent which comprises melting it with copper 0.5 to 0.9 per cent, nickel 0.1 to 0.35 per cent, molybdenum 0.4 to 0.75 per cent, chromium 0.1 to 0.3 per cent, manganese 0.5 to 1.0 per cent, adding zirconium 100 0.5 per cent and titanium 0.2 per cent to the melt and initiating a combination of the oxide impurities with the zirconium and titanium by the addition of an oxidizing agent selected from the group consisting of sodium bichromate, potassium bichromate, potassium chlorate, sodium nitrate, potassium permanganate and sodium perborate. 105
18. The method of treating iron having a carbon content not greater than 0.5 per cent which comprises melting it with copper 0.5 to 0.9 per cent, nickel 0.1 to 0.35 per cent, molybdenum 0.4 to 0.75 per cent, chromium 0.1 to 0.3 per cent, silicon 0.2 to 0.5 percent, manganese 0.5 to 0.1 per cent, adding zirconium in an amount substantially 110 0.5 per cent and titanium in an amount substantially 0.2 per cent and then initiating a combination of the oxide impurities with the zirconium and titanium by the addition of a trace of an oxidizing agent selected from the group 115 consisting of sodium bichromate, potassium bichromate, potassium chlorate, sodium nitrate, potassium permanganate and sodium perborate. 120
19. A method of treating iron having a carbon content not greater than 0.5 per cent which comprises melting it with copper 0.03 to 7 per cent, nickel 0.1 to 0.35 per cent, molybdenum 0.75 to 1.5 per cent, chromium 0.5 to 1.0 per cent, silicon 0.8 to 1.2 per cent, manganese 0.8 to 1.2 per cent, boron a trace, tungsten 0.3 to 0.6 per cent, 130 vanadium 0.1 to 0.2 per cent and cobalt a trace, adding zirconium 0.2 to 0.5 per cent and titanium 0.2 to 0.5 per cent and then initiating a combination of the oxide impurities with the zirconium and titanium by a trace of an oxidizing agent selected from the group consisting of sodium bichromate, potassium bichromate, potassium chlorate, sodium nitrate, potassium permanganate and sodium perborate. 135
- 140
- 145